

(No Model.)

E. T. THOMAS.

NUMBERING SEWING MACHINE CASTINGS.

No. 251,745.

Patented Jan. 3, 1882.

Fig:1.



Fig:2.



Fig. 3.



Witnesses.

*G. F. Connor.  
Arthur Reynolds.*

Inventor.

*Eddy T. Thomas,  
by Crosby & Gregory Attys.*

# UNITED STATES PATENT OFFICE.

EDDY T. THOMAS, OF NEW YORK, N. Y.

## NUMBERING SEWING-MACHINE CASTINGS.

SPECIFICATION forming part of Letters Patent No. 251,745, dated January 3, 1882.

Application filed April 1, 1881. (No model.)

*To all whom it may concern:*

Be it known that I, EDDY T. THOMAS, of New York, county of New York, and State of New York, have invented an Improvement in 5 Numbering Sewing-Machine Castings, of which the following description, in connection with the accompanying drawings, is a specification.

This invention has for its object to provide sewing-machine and other castings—as, for instance, the frame or arm of the machine—with chilled or hardened figures, which cannot be readily cut away with a chisel or file, as would be the case were the said figures made of un-chilled cast or malleable metal.

15 The invention consists in castings having designating characters—such as numbers, figures, letters, &c.—chilled thereupon in the casting, as hereinafter claimed.

To make castings which include my invention, I place in the loam in the flask an iron 20 chill-plate, against which the molten metal is poured into the said flask when casting the frame or other part to be cast runs, thereby hardening or chilling that portion of the molten metal which comes in contact with the said 25 chill-plate. This chill-plate will have cut into it the figures to be produced upon that part of the sewing-machine which is to be cast in the flask; but, if desired, I may make the outlines 30 of the figures in a thin layer of loam next the chill-plate, a portion of the chill-plate being exposed, to permit the molten metal forming the figures to come in contact with it.

Figure 1 represents, in longitudinal section, 35 a flask containing a chill-plate and a pattern, which in practice will correspond in shape with the part of a sewing or other machine which it is desired to reproduce as a casting. Fig. 2 is a similar view of a modification. Fig. 40 3 is a top plan view of the bed or frame, with the arm removed, of a sewing-machine numbered in accordance with my invention.

45 Referring to Fig. 1, *a b* represent the upper and lower portions, and *c* the board, of a molder's flask of usual construction.

I first lay the pattern *f* upon the board *c*, and fill the part *b* of the flask as deep with loam as the thickness of the pattern. After this I place the chill-plate *d* on the pattern and fill the part 50 *b* of the flask, and then I invert the part *b* on the board *c*, as in the drawings Fig. 1. This

chill-plate *d* is provided with figures or characters in intaglio; but they may, if desired, be in relief. The loam in the inverted part *b* is then sanded, the top part, *a*, is applied to the flask, and the loam *g* is filled in and provided with run-holes *h i* in the usual manner. The parts having all been properly tamped, the flask, Fig. 1, will be separated to remove the pattern *f*, leaving the chill-plate *d*, however, in the 60 flask. After this the molten metal will be poured into the run-holes, and will conform itself in shape to the space left in the flask by the pattern, and running against the cold surface of the chill-plate *d*, and, entering the recesses in its face, made in the form of figures, will become chilled at such points, leaving a series of chilled figures upon the cast-metal part of the frame-work of the machine—figures 65 so hard or so thoroughly chilled that they cannot be chipped or filed off as were the figures 70 on the frame-work produced by being cast in loam.

In Fig. 3 I have shown a bed or frame, *k*, of a sewing-machine with the number *l* thereof 75 cast upon it in chilled figures.

Providing a sewing-machine casting in this way with chilled figures is a matter of considerable importance, as it enables manufacturers of sewing-machines to keep track of the 80 various machines put out by their agents to parties who pay but small installments thereon, and then subsequently deface the numbers in order that the machines, partly paid for, may not be traced when passed by them 85 into other hands. These chill-numbers are a great safeguard to manufacturers, and prevent dishonest purchasers from disposing of machines which have not yet fully become their 90 own property.

It is obvious that, instead of forming the figures directly in the chill-plate *d*, I may place a thin layer of loam between the chill-plate *d* and pattern *f*, as in Fig. 2, and when the pattern is removed I may indent or impress into and through the said thin layer of loam upon the chill-plate *d*, by means of type or otherwise, the figures or characters which it is desired to have produced in the casting to be made in the flask. By forming the said figures or characters in the said thin layer of loam, so as to 95 cut through the said layer to the surface of the 100

plate *d*, the molten metal poured into the flask will come in contact with the chill-plate *d*, as before described, and be chilled at such points, thus producing chilled figures in the casting.

5 I claim—

A casting having an unchilled body and chilled designating characters in one piece with the body, as and for the purpose set forth.

In testimony whereof I have signed my name to this specification in the presence of two subscribing witnesses.

EDDY T. THOMAS.

Witnesses:

SPENCER C. DOTY,  
SAM'L. D. TOMPKINS.